

## UNITED STATES PATENT OFFICE

2,302,066

## TEXTILE PRODUCT

Richard R. Sitaler, Cumberland, Md., assignor to  
Celanese Corporation of America, a corporation  
of Delaware

No Drawing. Application April 25, 1940,  
Serial No. 331,661

5 Claims. (Cl. 66—202)

This invention relates to the knitting of yarns and relates more particularly to the knitting of yarns composed of stabilized fibers.

An object of this invention is the improvement of the knitting qualities of stabilized yarns.

Another object of this invention is to improve said knitting qualities so that garments and fabrics knitted therefrom will have a soft hand and will be free of defects.

Other objects of this invention will appear hereinafter from the following detailed description.

In the mechanical knitting of yarn, various articles may be produced. By the proper arrangement of the needles and their actuating mechanism sweaters, socks, cloth, gloves and various other articles of apparel may be knitted. These articles may be knitted in a single solid shade or, by varying the color of the yarn and the manner in which it is knitted into the article, a patterned effect may be achieved composed of two or more colors. Likewise, the stitch used in knitting the article or garment may also be varied and an unlimited number of effects may be achieved.

Various kinds of yarns may be used in knitting, depending upon the type of garment or article being knitted and the purpose for which it is to be used. Among the most desirable yarns used for knitting are those which are known as artificial silks. These synthetic yarns may be prepared by any one of a number of different processes and the yarns in commercial use today are identified as either viscose, cuprammonium, nitro-cellulose or cellulose acetate art silks, depending upon the process used for their manufacture. Besides the cellulose acetate, other organic derivatives of cellulose may be used for the production of artificial yarn, such as cellulose ethers and cellulose esters. Although these yarns find extensive commercial application when in continuous filament form, they are particularly desirable and attractive for certain special uses when the yarns are in stabilized form. By this stabilizing process the continuous filamentary character of the yarn is changed so that it resembles a yarn spun from staple fiber. This effect is achieved by severing different filaments comprising the yarn at different places along their lengths by controllably cutting or abrading the yarn. The resulting yarn is then composed of short lengths of filaments, the length of filament being varied as desired during the severing operation. This stabilized yarn, while resembling, in appearance, yarn spun from staple

fibers, is more durable than the latter in that it retains the highly desirable serimetric properties of continuous filament yarn.

Cloth having a very soft and full appearance may be woven from such yarns but when it is desired to produce a knitted fabric from such stabilized yarns serious difficulties are sometimes encountered. Since the yarn is composed of comparatively short lengths of filaments, individual filaments occasionally work loose and produce a substantial amount of lint and wild filaments. As a result the operation of the knitting machine is seriously hampered and a substantial percentage of articles knitted must be discarded, being unsatisfactory because of the holes which are due to bursting out in knitting or the dropping of stitches. Various attempts to overcome these difficulties have been made but a rather substantial proportion of articles knitted were still unacceptable commercially.

I have now discovered that continuous filament yarns which have been stabilized may be successfully knitted on various commercial knitting machines if continuous filament yarns having a 25 denier per filament of less than about 2.0 are used for the production of the stabilized yarn. Preferably I employ a continuous filament yarn having a denier per filament of about 1.5. When using stabilized yarns produced from such continuous filament yarn, plain stitches, rib stitches, tuck stitches and a wide variety of other types of stitches and patterns may be knitted therewith, the resulting knitted articles exhibiting a high degree of uniformity and freedom from 35 defects (holes).

The length of filament contained in these stabilized yarns may be varied as desired by varying the adjustment of the stabilizing mechanism. Yarns in which the staple length varies 40 from 3 inches to about 20 inches are very satisfactory, but I preferably use yarns in which the staple length is from about 10 to about 11 inches.

Highly twisted stabilized yarns, as well as yarns having a low degree of twist, may be used for 45 knitting. Yarns in which the number of turns per inch varies from about 3 to about 15 are suitable, but I prefer to use the low denier yarns which have about 5 turns per inch.

While these low denier per filament stabilized 50 yarns knit satisfactorily in the absence of any lubricant, for some types of stitches the addition of about 1% to about 2.5% of a lubricant may be desired. Lubricants such as sulphonated olive oil mixed with sperm oil and mineral oil are suitable and the lubricant may be applied to the

yarn by means of a wick, for instance, or in any other suitable manner at any stage in the manufacture of the yarn prior to knitting. Application of lubricant at the metier yields excellent results. Also, the yarn may be dyed any suitable shade prior to knitting or the article may be dyed after it is knitted. The present invention is applicable to lustrous yarns as well as to lusterless yarns.

It is to be understood that the foregoing detailed description is merely given by way of illustration and that many variations may be made therein without departing from the spirit of my invention.

Having described my invention, what I desire to secure by Letters Patent is:

1. Method of producing knitted fabric, which comprises knitting into a fabric yarn prepared by stabilizing an artificial continuous filament yarn in which the denier per filament is substantially 1.5.

2. Method of producing knitted fabric, which comprises knitting into a fabric yarn prepared

by stabilizing an artificial continuous filament yarn in which the denier per filament is substantially 1.5, said yarn being lubricated prior to the knitting operation.

3. Method of producing knitted fabric, which comprises knitting into a fabric yarn prepared by stabilizing an artificial continuous filament yarn in which the denier per filament is substantially 1.5, said yarn containing from 1.5% to 2.5% of a yarn lubricant.

4. Method of producing knitted fabric, which comprises knitting into a fabric yarn prepared by stabilizing continuous filament yarn having a basis of an organic derivative of cellulose and in which the denier per filament is substantially 1.5.

5. Method of producing knitted fabric, which comprises knitting into a fabric yarn prepared by stabilizing continuous filament yarn having a basis of cellulose acetate and in which the denier per filament is substantially 1.5.

RICHARD R. SITZLER.